



US007354688B2

(12) **United States Patent**  
Silence et al.

(10) **Patent No.:** US 7,354,688 B2  
(45) **Date of Patent:** Apr. 8, 2008

(54) **TONER COMPOSITIONS WITH SURFACE ADDITIVES**

(75) Inventors: **Scott M. Silence**, Fairport, NY (US); **Joo T. Chung**, Webster, NY (US); **Juan A. Morales-Tirado**, West Henrietta, NY (US)

(73) Assignee: **Xerox Corporation**, Norwalk, CT (US)

(\*) Notice: Subject to any disclaimer, the term of this patent is extended or adjusted under 35 U.S.C. 154(b) by 407 days.

(21) Appl. No.: **10/980,234**

(22) Filed: **Nov. 4, 2004**

(65) **Prior Publication Data**

US 2006/0093941 A1 May 4, 2006

(51) **Int. Cl.**

**G03G 9/08** (2006.01)

(52) **U.S. Cl.** ..... **430/108.3**; 430/108.4; 430/108.6; 430/108.7; 430/137.1

(58) **Field of Classification Search** ..... 430/108.4, 430/108.6, 108.7, 108.3, 137.1

See application file for complete search history.

(56) **References Cited**

U.S. PATENT DOCUMENTS

|             |         |                  |
|-------------|---------|------------------|
| 3,590,000 A | 6/1971  | Palermiti et al. |
| 4,265,990 A | 5/1981  | Stolka et al.    |
| 4,298,672 A | 11/1981 | Lu               |
| 4,338,390 A | 7/1982  | Lu               |
| 4,558,108 A | 12/1985 | Alexandru et al. |
| 4,563,408 A | 1/1986  | Lin et al.       |

|                   |         |                                  |
|-------------------|---------|----------------------------------|
| 4,584,253 A       | 4/1986  | Lin et al.                       |
| 4,585,884 A       | 4/1986  | Lin et al.                       |
| 4,883,736 A       | 11/1989 | Hoffend et al.                   |
| 4,935,326 A       | 6/1990  | Creatura et al.                  |
| 4,937,166 A       | 6/1990  | Creatura et al.                  |
| 5,352,556 A       | 10/1994 | Mahabadi et al.                  |
| 5,545,501 A       | 8/1996  | Tavernier et al.                 |
| 6,004,714 A       | 12/1999 | Ciccarelli et al.                |
| 6,017,668 A       | 1/2000  | Young et al.                     |
| 6,071,665 A       | 6/2000  | Dickerson et al.                 |
| 6,087,059 A *     | 7/2000  | Duggan et al. .... 430/108.4     |
| 6,103,440 A       | 8/2000  | Lohr                             |
| 6,124,071 A       | 9/2000  | Lin et al.                       |
| 6,177,221 B1 *    | 1/2001  | Maniar et al. .... 430/111.3     |
| 6,399,264 B1 *    | 6/2002  | Ogata et al. .... 430/108.6      |
| 2004/0063018 A1   | 4/2004  | Silence et al.                   |
| 2004/0110079 A1 * | 6/2004  | Matsushima et al. .... 430/110.4 |
| 2006/0003244 A1 * | 1/2006  | Grande et al. .... 430/108.6     |

FOREIGN PATENT DOCUMENTS

GB 1442835 7/1976

OTHER PUBLICATIONS

Material Safety and Data Sheet for "SMT5103" (Jul. 30, 2004). Specification for "DTMS Silica", p. 1.

\* cited by examiner

Primary Examiner—Christopher RoDee

(74) Attorney, Agent, or Firm—Oliff & Berridge, PLC

(57) **ABSTRACT**

A toner composition includes a binder, a colorant, and a surface additive package including a polydimethylsiloxane surface treated silica, a surface treated titania, and calcium sterate. The toner composition provides improved triboelectric charging properties.

16 Claims, 2 Drawing Sheets



FIG. 1



FIG. 2

## 1

## TONER COMPOSITIONS WITH SURFACE ADDITIVES

## BACKGROUND OF THE INVENTION

## 1. Field of Invention

This invention relates generally to toner compositions having improved properties that are provided by improved surface additives. More particularly, the present invention relates to toner and developer compositions where the toner particles have an external additive mixture of treated silica, treated titania, and calcium stearate. The invention also relates to developers containing such toners, processes for making such toners and developers, and methods for generating developed images with such toners and developers.

## 2. Description of Related Art

In electrophotography, a photoreceptor containing a photoconductive insulating layer on a conductive layer is imaged by first uniformly electrostatically charging its surface. The photoreceptor is then exposed to a pattern of activating electromagnetic radiation, such as light. The radiation selectively dissipates the charge in the illuminated areas of the photoconductive insulating layer while leaving behind an electrostatic latent image in the non-illuminated areas. This electrostatic latent image may then be developed to form a visible image by depositing finely divided toner particles on the surface of the photoconductive insulating layer. The resulting visible image may then be transferred from the photoconductor to a support, such as transparency or paper. This imaging process may be repeated many times.

Various toner compositions for such a printing system are well known in the art, and have been produced having a wide range of additives and constituent materials. Generally, however, the toner particles include a binding material such as a resin, a colorant such as a dye and/or a pigment, and any of various additives to provide particular properties to the toner particles.

U.S. Pat. No. 5,545,501 describes an electrostatographic developer composition comprising carrier particles and toner particles with a toner particle size distribution having a volume average particle size (T) such that  $4 \mu\text{m} \leq T \leq 12 \mu\text{m}$ , and an average charge (absolute value) pro diameter in femtocoulomb/10  $\mu\text{m}$  ( $C_T$ ) after triboelectric contact with the carrier particles such that  $1 \text{ fC}/10 \mu\text{m} \leq C_T \leq 10 \text{ fC}/10 \mu\text{m}$ , and wherein (i) the carrier particles have a saturation magnetization value,  $M_{sat}$ , expressed in Tesla (T) such that  $M_{sat} \geq 0.30 \text{ T}$ ; (ii) the carrier particles have a volume average particle size ( $C_{avg}$ ) such that  $30 \mu\text{m} \leq C_{avg} \leq 60 \mu\text{m}$ ; (iii) the volume based particle size distribution of the carrier particles has at least 90 percent of the particles having a particle diameter C such that  $0.5 C_{avg} \leq C \leq 2 C_{avg}$ ; (iv) the volume based particles size distribution of the carrier particles comprises less than b percent particles smaller than  $25 \mu\text{m}$  wherein  $b = 0.35 \times (M_{sat})^2 \times P$  with  $M_{sat}$ : saturation magnetization value,  $M_{sat}$ , expressed in T and P, the maximal field strength of the magnetic developing pole expressed in kA/m, and (v) the carrier particles comprise a core particle coated with a resin coating in an amount (RC) such that 0.2 percent w/w  $\leq RC \leq 2$  percent w/w, see the Abstract. This patent indicates that the developers thereof can achieve images when a latent image is developed with a fine hair magnetic brush, see for example, column 4, lines 7 to 17.

Nevertheless, there continues to be a need for a set of developers comprised of toners and carriers that possess a combination of properties such that when used to develop a latent image on the surface of a photoreceptor, preferably in an image-on-image device, and more specifically, in such a

## 2

device also utilizing a hybrid scavengelss development system, the color image produced exhibits a quality analogous to that achieved in offset lithography. Further, there is a need for toners and developers wherein a toner additive does not substantially interact with fuser oils, fuser rolls, and the like to thereby, for example, increase the usable life, for example from about 200,000 prints to about 1,000,000 prints, of fuser devices, such as fuser rolls, and wherein the toners and developers thereof possess excellent triboelectrical, conductivity, and developability characteristics.

One approach for addressing these needs is shown in U.S. Patent Publication No. 20040063018, the entire disclosure of which is incorporated herein by reference. In the publication toner and developer compositions are disclosed that comprise at least one binder in an optional amount of from about 85 to about 99 percent by weight, at least one colorant in an optional amount of from about 0.5 to about 15 percent by weight, and calcium stearate in an optional amount of from about 0.05 to about 2 percent by weight.

Despite the various attempts to provide toner and developer compositions for providing high quality print results, problems still remain. For example, as the end-user demands for higher quality prints increases, and as the printing apparatuses are utilized in a wider variety of environments, increasing demands are being placed on the printing apparatuses and the toner and developer compositions. Thus, while particular printing apparatuses and toner and developer compositions are designed to provide adequate results over a wide range of customer job types and operating conditions, those parameters are being widened to increase the performance demands.

One such demand is the triboelectric charging values of the toner and developer compositions. The conventional range for developer triboelectric charging values is generally accepted to be from about 25 to about 50  $\mu\text{C}/\text{g}$ . This range is limited on the lower end by macrouniformity (half-tone mottle), dirt, emissions, spittings, and gaps and traps defects; and is limited on the higher end by transfer image quality defects. While this range provides high quality print results for a large proportion of the end-users, there exists a "tail" of end-users at both ends, where operating conditions provide less than superior print results. These tail operation conditions are driven primarily by inherent variations in the machines and compositions as produced, as well as variation in the developer toner concentration, ambient temperature and relative humidity conditions, and age of the developer components. Relative humidity can be somewhat controlled, by using an environmental unit in the print cavity to dehumidify the print cavity and to control humidity on the high end, and a humidifier in the room housing the printing apparatus to control humidity on the low end. However, this requirement for the end-user to provide humidification control is difficult in some cases and thus is undesirable.

## SUMMARY OF THE INVENTION

This invention addresses some or all of the above problems, and others, by providing toner and developer compositions where the toner composition includes a novel additive package to control triboelectric charging to within a desired range. This invention thus relates to toners, developers containing toners, processes thereof, and methods for generating developed images with, for example, high print quality.

It is a feature of the present invention to provide toner and developer compositions having a set of properties such that

the developers containing such toners can achieve xerographically produced images having high print quality.

It is a still further feature of the invention to provide processes for the preparation of the toners and developers with certain consistent, and predictable properties.

Furthermore, another feature of the present invention relates to the selection of calcium stearate as a lubricant component for toners and developers thereof that, in combination with other components of an external additive package, permit the toner to exhibit a greatly reduced sensitivity of triboelectric charging properties to relative humidity, optimize the triboelectric charging response to age of the toner and developer, and provide a sufficiently high triboelectric charge to allow tenability of the developer by appropriate carrier choice.

More particularly, in embodiments, the present invention provides a toner composition comprising:

a binder,  
a colorant, and

a surface additive package comprising a polydimethylsiloxane surface treated silica, a surface treated titania, and calcium stearate.

The present invention also provides developers including such a toner composition, and methods for making and using such toner and developer compositions.

#### BRIEF DESCRIPTION OF THE DRAWINGS

These and other advantages and features of this invention will be apparent from the following, especially when considered with the accompanying drawings, in which:

FIG. 1 is a graph showing measured triboelectric charge for control developers and developers according to an embodiment of the invention, as a function of different external additive packages.

FIG. 2 is a graph showing measured triboelectric charge for control developers and developers according to an embodiment of the invention, as a function of simulated toner age.

#### DETAILED DESCRIPTION OF PREFERRED EMBODIMENTS

According to the present invention, a toner is provided that includes at least a binder, a colorant, and a surface additive package. The surface additive package comprises a polydimethylsiloxane (PDMS) surface treated silica, a surface treated titania, and calcium stearate. The additive package is used as an external additive to the toner composition. That is, the toner particles per se are first formed, followed by mixing of the toner particles with the materials of the additive package. The result is that the additive package generally coats or adheres to external surfaces of the toner particles, rather than being incorporated into the bulk of the toner particles.

The first component of the additive package is a polydimethylsiloxane (PDMS) surface treated silica. Preferably, the polydimethylsiloxane (PDMS) surface treated silica used in embodiments is a polydimethylsiloxane (PDMS) surface treated fumed silica.

Conventional surface treated silica materials are known and include, for example, TS-530 from Cabosil Corporation, with an 8 nanometer particle size and a surface treatment of hexamethyldisilazane; NA5OHS silica, obtained from DeGussa/Nippon Aerosil Corporation, coated with a mixture of HMDS and aminopropyltriethoxysilane; DTMS (decyltrimethoxysilane) silica, obtained from Cabot Corporation,

comprised of a finned silica silicon dioxide core L90 coated with DTMS; H2050EP, obtained from Wacker Chemie, coated with an amino functionalized organopolysiloxane; and the like. Such conventional surface treated silicas are applied to the toner surface for toner flow, triboelectric charge enhancement, admix control, improved development and transfer stability, and higher toner blocking temperature.

However, the present inventors have found that a specific surface treated silica, a silica surface treated with polydimethylsiloxane (PDMS), unexpectedly provides superior performance results to the final toner composition when used in combination with a surface treated titania and calcium stearate in an additive package. In particular, the present inventors have found that the polydimethylsiloxane (PDMS) surface treated silica, when used in combination with a surface treated titania and calcium stearate in an additive package, provides higher triboelectric charge in different temperature/humidity environments, and provides different and desirable performance response in printing environments. For example, conventional surface treated silicas are known to exhibit triboelectric charging effects in different temperature/humidity environments. That is, it is known that for most surface treated silicas, as the concentration of the surface treated silica is decreased, the triboelectric charge increases in both the relatively higher humidity B-zone (70° F., 50% RH) and the relatively lower humidity J-zone (70° F., 10% RH). However, the present inventors unexpectedly discovered that a PDMS-surface treated silica exhibits different results—namely, as the concentration of the PDMS-surface treated silica is decreased, the triboelectric charge increases in the B-zone, but substantially decreases in the J-zone. This allows for more specific tailoring of triboelectric charging properties, for example, such that the triboelectric charge does not change substantially between the B and J zones (as relative humidity charges).

Specific examples of suitable PDMS-surface treated silicas include, for example, but are not limited to, RY50, NY50, RY200, RY200S and R202, all available from Nippon Aerosil, and the like.

The polydimethylsiloxane (PDMS) surface treated silica is preferably present in an amount of from about 1 to about 10 percent by weight, based on a weight of the toner particles without the additive (i.e., in an amount of from about 1 to about 10 parts by weight additive per 100 parts by weight toner particle). More preferably, in embodiments, the PDMS surface treated silica is present in an amount of from about 1.5 or from about 2 to about 5.5 or to about 6 percent by weight, such as from about 2.3 or about 2.5 to about 4.3 or about 4.5 percent by weight. However, weight percents outside of these ranges can be used, if desired.

Preferably, according to embodiments of the invention, the polydimethylsiloxane (PDMS) surface treated silica is the only surface treated silica present in the toner composition. Alternatively, for example where small amounts of other silicas are introduced into the toner composition for other purposes, such as to assist toner particle classification and separation, the polydimethylsiloxane (PDMS) surface treated silica is the only xerographically active surface treated silica present in the toner composition. Any other incidentally present silica thus does not significantly affect any of the xerographic printing properties. Preferably, the polydimethylsiloxane (PDMS) surface treated silica is the only surface treated silica present in the additive package applied to the toner composition.

## 5

The second component of the additive package is a surface treated titania. Preferably, the surface treated titania used in embodiments is a hydrophobic surface treated titania.

Conventional surface treated titania materials are known and include, for example, metal oxides such as  $TiO_2$ , for example MT-3103 from Tayca Corp. with a 16 nanometer particle size and a surface treatment of decylsilane; SMT5103, obtained from Tayca Corporation, comprised of a crystalline titanium dioxide core MT500B coated with DTMS; P-25 from Degussa Chemicals with no surface treatment; STT100H, an isobutyltrimethoxysilane (I-BTMS) treated hydrophobic titania obtained from Titan Kogyo Kabushiki Kaisha (IK Inabata America Corporation, New York); and the like. Such surface treated titania are applied to the toner surface for improved relative humidity (RH) stability, triboelectric charge control and improved development and transfer stability.

However, the present inventors have found that specific surface treated titania materials unexpectedly provides superior performance results to the final toner composition. Thus, while any of the surface treated titania may be used in the external additive package, in embodiments it is preferred that the material be a "large" surface treated titania (i.e., one having an average particle size of from about 30 to about 50 nm, or from about 35 to about 45 nm, particularly about 40 nm). In particular, the present inventors have found that the preferred surface treated titania provides one or more of better cohesion stability of the toners after aging in the toner housing, and higher toner conductivity, which increases the ability of the system to dissipate charge patches on the toner surface.

Specific examples of suitable surface treated titanias include, for example, but are not limited to, STT100H, an isobutyltrimethoxysilane (I-BTMS) treated hydrophobic titania obtained from Titan Kogyo Kabushiki Kaisha (IK Inabata America Corporation, New York); SMT5103, obtained from Tayca Corporation, comprised of a crystalline titanium dioxide core MT500B coated with DTMS (decyltrimethoxysilane); and the like. The STT100H is particularly preferred, in some embodiments.

The silicas and titanias should more specifically possess a primary particle size greater than approximately 30 nanometers, preferably of at least 40 nanometers, with the primary particles size measured by, for instance, transmission electron microscopy (TEM) or calculated (assuming spherical particles) from a measurement of the gas absorption, or BET, surface area. Titania is found to be especially helpful in maintaining development and transfer over a broad range of area coverage and job run length. The silica and titania are more specifically applied to the toner surface with the total coverage of the toner ranging from, for example, as low as about 60% or about 70% to as high as about 200% theoretical surface area coverage (SAC), preferably from about 70% or about 100% to about 200% theoretical surface area coverage (SAC), where the theoretical SAC (hereafter referred to as SAC) is calculated assuming all toner particles are spherical and have a diameter equal to the volume median diameter of the toner as measured in the standard Coulter Counter method, and that the additive particles are distributed as primary particles on the toner surface in a hexagonal closed packed structure. Another metric relating to the amount and size of the additives is the sum of the "SAC $\times$ Size" (surface area coverage times the primary particle size of the additive in nanometers) for each of the silica and titania particles, or the like, for which all of the additives should, more specifically, have a total SAC $\times$ Size range of,

## 6

for example, from about 2,400 to about 8,000, preferably in embodiments from about 4,500 to about 7,200. The ratio of the silica to titania particles is generally from about 50 percent silica/50 percent titania to about 85 percent silica/15 percent titania (on a weight percentage basis), although the ratio may be larger or smaller than these values provided that the features of the invention are achieved.

The surface treated titania is preferably present in an amount of from about 0.1 to about 5 percent by weight, 10 based on a total weight of the toner particles. More preferably, in embodiments, the surface treated titania is present in an amount of from about 0.2 or from about 0.3 to about 1.0 or to about 2.0 percent by weight. However, weight percents outside of these ranges can be used, if desired.

15 Preferably, according to embodiments of the invention, only one surface treated titania is present in the toner composition. That is, in some embodiments, it is preferred that only one kind of surface treated titania be present, rather than a mixture of two or more different surface treated titanias.

20 The third component of the additive package is calcium stearate.

Calcium stearate is used in the additive package of the 25 present invention primarily to provide lubricating properties. Also, the calcium stearate can provide developer conductivity and triboelectric charge enhancement, both due to its lubricating nature. In addition, calcium stearate has been found to enable higher toner charge and charge stability by 30 increasing the number of contacts between toner and carrier particles.

Any suitable calcium stearate can be used in the additive 35 package. However, it is preferred that the calcium stearate, preferably commercially available, has greater than about 85 percent purity, for example from about 85 to about 100 percent purity. For example, the 85 percent pure calcium stearate preferably has less than 12 percent calcium oxide and free fatty acid by weight, and less than 3 percent moisture content by weight. The calcium stearate also preferably has an average particle diameter of about 7 microns. 40 A suitable calcium stearate meeting these preferred parameters is available from Ferro Corporation (Cleveland, Ohio). Examples include, but are not limited to, SYNPRO® Calcium Stearate 392A and SYNPRO® Calcium Stearate NF Vegetable. Most preferred is a commercially available calcium stearate with greater than 95 percent purity (less than 0.5 percent calcium oxide and free fatty acid by weight, and less than 4.5 percent moisture content by weight), and which calcium stearate has an average particle diameter of about 2 microns and is available from NOF Corporation (Tokyo, Japan).

45 The calcium stearate is preferably present in an amount of from about 0.01 to about 10 percent by weight, based on a total weight of the toner particles. More preferably, in embodiments, the calcium stearate is present in an amount of from about 0.05 or from about 0.1 to about 2.5 or to about 50 5.0 percent by weight. However, weight percents outside of these ranges can be used, if desired.

55 Preferably, according to embodiments of the invention, the calcium stearate is the only metal carboxylate, or at least 60 the only metal stearate, present in the toner composition. Thus, for example, it is preferred in some embodiments that no other metal carboxylates, such as zinc stearate, be present in the toner composition.

The components of the additive package are selected to 65 enable superior toner flow properties, high toner charge and charge stability. The surface treatments on the silica and titania, the relative amounts of the silica and titania (for

example about 90 percent silica:about 10 percent titania (all percentages are by weight) to about 10 percent silica:about 90 percent titania), and the amount of calcium stearate can be manipulated to provide a range of toner charge values. For example, toner charge values can be provided ranging from about 10  $\mu$ C/g to about 60  $\mu$ C/g, as measured by the standard Faraday Cage technique.

Thus, for example, in embodiments, the toners contain from, for example, about 1 to about 5 weight percent PDMS surface treated silica, about 0.2 to about 1.5 weight percent surface treated titania, and about 0.05 to about 0.5 weight percent calcium stearate. Exemplary toner compositions may thus include, for example, about 3.3 weight percent PDMS surface treated silica, about 0.9 weight percent surface treated titania, and about 0.1 weight percent calcium stearate, or about 4.3 weight percent PDMS surface treated silica, about 0.9 weight percent surface treated titania, and about 0.1 or 0.2 weight percent calcium stearate. Of course, these range are exemplary only, and values outside these ranges can be used, in embodiments.

For further enhancing the positive charging characteristics of the toner developer compositions, and as optional components there can be incorporated into the toner or on its surface charge enhancing additives inclusive of alkyl pyridinium halides, reference U.S. Pat. No. 4,298,672, the disclosure of which is totally incorporated herein by reference; organic sulfate or sulfonate compositions, reference U.S. Pat. No. 4,338,390, the disclosure of which is totally incorporated herein by reference; distearyl dimethyl ammonium sulfate; bisulfates, and the like, and other similar known charge enhancing additives. Also, negative charge enhancing additives may also be selected, such as aluminum complexes, like BONTRON E-88®, and the like. These additives may be incorporated into the toner in an amount of from about 0.1 percent by weight to about 20 percent by weight, and more specifically from about 1 to about 3 percent by weight.

The toner compositions of the present invention, in addition to including the above-described additive package, generally also include at least a toner resin and a colorant. In addition, the toner compositions can include one or more conventional additives, including but not limited to, optional charge enhancing additives and optional waxes, especially low molecular weight waxes with an Mw of, for example, from about 1,000 to about 20,000. Suitable toner compositions, which can be modified to include the above-described external additive package of the present invention, include those toner compositions disclosed in, for example, U.S. Pat. Nos. 6,004,714, 6,017,668, 6,071,665, 6,087,059, 6,103, 440, and 6,124,071, and U.S. Patent Publication No. 20040063018, the entire disclosures of which are incorporated herein by reference. The toner compositions can generally be prepared by any known technique, such as by admixing and heating resin particles, colorant, and optional additives other than the above-described surface additive in a suitable toner extrusion device, such as the ZSK58 available from Werner Pfleiderer, following by removing the formed toner composition from the device. Subsequent to cooling, the toner composition is subjected to grinding utilizing, for example, a Sturtevant micronizer for the purpose of achieving toner particles with a desired volume median diameter of, for example, less than about 25 microns, and preferably of from about 6 to about 12 microns, which diameters are determined by a Coulter Counter. Subsequently, the toner compositions can be classified utilizing, for example, a Donaldson Model B classifier for the purpose of removing fines, that is toner particles having a

volume median diameter of less than about 4 microns. Thereafter, the above-described external additive package and other optional surface additives can be added to the toner composition by blending the additives with the obtained toner particles.

As the toner (or binder) resin, any of the convention toner resins can be used. Illustrative examples of such suitable toner resins include, for example, thermoplastic resins such as vinyl resins in general or styrene resins in particular, and 10 polyesters. Examples of suitable thermoplastic resins include, but are not limited to, styrene methacrylate; polyolefins; styrene acrylates, such as PSB-2700 obtained from Hercules-Sanyo Inc.; polyesters, styrene butadienes; 15 crosslinked styrene polymers; epoxies; polyurethanes; vinyl resins, including homopolymers or copolymers of two or more vinyl monomers; and polymeric esterification products of a dicarboxylic acid and a diol comprising a diphenol. Other suitable Vinyl monomers include, but are not limited to, styrene; p-chlorostyrene; unsaturated mono-olefins such 20 as ethylene, propylene, butylene, isobutylene and the like; saturated mono-olefins such as vinyl acetate, vinyl propionate, and vinyl butyrate; vinyl esters such as esters of monocarboxylic acids including methyl acrylate, ethyl acrylate, n-butyl acrylate, isobutyl acrylate, dodecyl acrylate, 25 n-octyl acrylate, phenyl acrylate, methyl methacrylate, ethyl methacrylate, and butyl methacrylate; acrylonitrile, methacrylonitrile, and acrylamide; mixtures thereof; and the like. In addition, crosslinked resins, including polymers, copolymers, and homopolymers of styrene polymers, may be selected.

For example, as one toner resin, there can be selected the esterification products of a dicarboxylic acid and a diol comprising a diphenol. These resins are illustrated, for example, in U.S. Pat. No. 3,590,000, the entire disclosure of 35 which is incorporated herein by reference. Other specific toner resins include, but are not limited to, styrene/methacrylate copolymers, and styrene/butadiene copolymers; Pliolites; suspension polymerized styrene butadienes, reference U.S. Pat. No. 4,558,108, the entire disclosure of which 40 is incorporated herein by reference; polyester resins obtained from the reaction of bisphenol A and propylene oxide; followed by the reaction of the resulting product with fumaric acid, and branched polyester resins resulting from the reaction of dimethylterephthalate, 1,3-butanediol, 1,2-45 propanediol, and pentaerythritol; reactive extruded resins, especially reactive extruded polyesters with crosslinking as illustrated in U.S. Pat. No. 5,352,556, the entire disclosure of which is incorporated herein by reference, styrene acrylates, and mixtures thereof. Also, waxes with a molecular weight Mw of from about 1,000 to about 20,000, such as 50 polyethylene, polypropylene, and paraffin waxes, can be included in, or on the toner compositions as fuser roll release agents.

The toner resin is generally present in any sufficient, but 55 effective amount. For example, the toner resin is generally present in an amount of from about 50 to about 95 percent by weight of the toner composition. More preferably, the toner resin is generally present in an amount of from about 70 to about 90 percent by weight of the toner composition.

The toner composition also generally includes a colorant. As desired, the colorant can be a dye, a pigment, a mixture 60 of a dye and a pigment, or two or more of them. As colored pigments, there can be selected, for example, various known cyan, magenta, yellow, red, green, brown, or blue colorants, or mixtures thereof. Specific examples of pigments include, but are not limited to, phthalocyanine HELIOGEN BLUE L6900™, D6840™, D7080™, D7020™, PYLAM OIL

BLUETM, PYLAM OIL YELLOWTM, PIGMENT BLUE 1TM, available from Paul Uhlich & Company, Inc., PIGMENT VIOLET 1TM, PIGMENT RED 48TM, LEMON CHROME YELLOW DCC 1026TM, E.D. TOLUIDINE REDTM and BON RED CTM available from Dominion Color Corporation, Ltd., Toronto, Ontario, NOVAPERM YELLOW FGLTM, HOSTAPERM PINK ETM from Hoechst, CINQUASIA MAGENTATA TM available from E.I. DuPont de Nemours & Company, Pigment Yellow 180, Pigment Yellow 12, Pigment Yellow 13, Pigment Yellow 14, Pigment Yellow 17, Pigment Blue 15, Pigment Blue 15:3, Pigment Red 122, Pigment Red 57:1, Pigment Red 81:1, Pigment Red 81:2, Pigment Red 81:3, and the like.

Generally, colored dyes and pigments that can be selected are cyan, magenta, or yellow pigments, and mixtures thereof. Examples of magentas that may be selected include, for example, 2,9-dimethyl-substituted quinacridone and anthraquinone dye identified in the Color Index as CI 60710, CI Dispersed Red 15, diazo dye identified in the Color Index as CI 26050, CI Solvent Red 19, and the like. Illustrative examples of cyans that may be selected include copper tetra(octadecyl sulfonamido) phthalocyanine, x-copper phthalocyanine pigment listed in the Color Index as CI 74160, CI Pigment Blue, and Anthrathrene Blue, identified in the Color Index as CI 69810, Special Blue X-2137, and the like. Illustrative examples of yellows that may be selected are diarylide yellow 3,3-dichlorobenzidine acetoacetanilides, a monoazo pigment identified in the Color Index as CI 12700, CI Solvent Yellow 16, a nitrophenyl amine sulfonamide identified in the Color Index as Foron Yellow SE/GLN, CI Dispersed Yellow 33 2,5-dimethoxy-4-sulfonanilide phenylazo-4'-chloro-2,5-dimethoxy acetoacetanilide, and Permanent Yellow FGL. Other soluble dyes, such as red, blue, green, and the like, can also be used, as desired.

Generally, the colorant is included in the toner composition in known amounts, for the desired color strength. For example, the above-described dyes and pigments, and others, can be included in the toner composition in any suitable amount, such as from about 1 to about 20 percent by weight of the toner composition. Preferably, the colorant is included in an amount of from about 2 to about 10 percent by weight of the toner composition.

If desired, such as to give the toner composition magnetic properties, magnetites can also be included in the toner composition, either for their magnetic properties, or for the colorant properties, or both. Suitable magnetites that can be used in the toner compositions of the present invention include, but are not limited to, a mixture of iron oxides (FeO.Fe<sub>2</sub>O<sub>3</sub>), including those commercially available as MAPICO BLACKTM. The magnetite can be present in the toner composition in any of various effective amounts, such as an amount of from about 10 percent by weight to about 75 percent by weight of the toner composition. Preferably, the magnetite is present in an amount of from about 30 percent to about 55 percent by weight of the toner composition.

There can be included in the toner compositions of the present invention charge additives as indicated herein in various effective amounts, such as from about 1 to about 15, and preferably from about 1 to about 3, percent by weight of the toner composition. Such suitable charge additives can include the above-described external additive package, or other charge additives well known in the art.

Furthermore, the toner compositions of the present invention can also include suitable waxes for their known effect. Suitable waxes include, but are not limited to, polypropy-

lenes and polyethylenes commercially available from Allied Chemical and Petrolite Corporation; Epolene N-15 commercially available from Eastman Chemical Products, Inc.; Viscol 550-P, a low weight average molecular weight polypropylene available from Sanyo Kasei K.K.; mixtures thereof, and the like. The commercially available polyethylenes selected possess, for example, a weight average molecular weight of from about 1,000 to about 1,500, while the commercially available polypropylenes utilized are believed to have a weight average molecular weight of from about 4,000 to about 7,000. Many of the polyethylene and polypropylene compositions useful in the present invention are illustrated in British Patent No. 1,442,835, the entire disclosure of which is incorporated herein by reference.

The wax can be present in the toner composition of the present invention in various amounts. However, generally these waxes are present in the toner composition in an amount of from about 1 percent by weight to about 15 percent by weight, and preferably in an amount of from about 2 percent by weight to about 10 percent by weight, based on the weight of the toner composition.

The toners of the present invention may also, in embodiments, contain polymeric alcohols, such as UNILINSTM, reference U.S. Pat. No. 4,883,736, the entire disclosure of which is incorporated herein by reference. The UNILINSTM products are available from Petrolite Corporation.

Developer compositions can be prepared by mixing the toners with known carrier particles, including but not limited to coated carriers, such as steel, ferrites, and the like, reference U.S. Pat. Nos. 4,937,166 and 4,935,326, the entire disclosures of which are incorporated herein by reference. The toner composition and carrier particles are generally mixed to include from about 2 percent toner concentration to about 8 percent toner concentration. The carriers can include coatings thereon, such as those illustrated in the above-referenced U.S. Pat. Nos. 4,937,166 and 4,935,326 patents, and other known coatings. There can be selected a single coating polymer, or a mixture of polymers. Additionally, the polymer coating or coatings may contain conductive components therein, such as carbon black in an amount for example, of from about 10 to about 70 weight percent, and preferably from about 20 to about 50 weight percent. Specific examples of coatings are fluorocarbon polymers, acrylate polymers, methacrylate polymers, silicone polymers, and the like.

A particularly preferred coated carrier for use in embodiments to make developer compositions is formed from 80  $\mu$ m steel core particles (such as those supplied by Hoeganaes North America Corporation) coated with about 0.2% (by wt.) of methylsilsesquioxane Silicone Resin and about 1.0% (by wt.) PMMA.

Imaging methods are also envisioned with the toners of the present invention. Suitable imaging methods that utilize toner particles are known in the art and include, for example, but are not limited to, the various patents mentioned herein as well as U.S. Pat. Nos. 4,585,884, 4,584,253, 4,563,408, and 4,265,990, the entire disclosures of which are incorporated herein by reference.

The toner compositions prepared according to the present invention provide excellent results in electrostatographic printing operations. In particular, the toner compositions, including the treated aerosil particles, possess good triboelectric charge properties, and good admix times.

In embodiments of the present invention, the toner compositions have a triboelectric charge of from about 15 to about 70  $\mu$ C/g. Preferably, the toner compositions have a

## 11

triboelectric charge of from about 25 to about 65  $\mu\text{C/g}$ , more preferably from about 30 to about 60  $\mu\text{C/g}$ .

## EXAMPLES

The invention will be illustrated in greater detail with reference to the following Examples and Comparative Examples, but the invention should not be construed as being limited thereto. In the following examples and comparative examples, all the "parts" are given by weight unless otherwise indicated.

## Comparative Example 1

## Black Toner with Zinc Stearate

A black toner is prepared by melt mixing together 5% by weight carbon black in a propoxylated bisphenol A fumarate resin having a gel content of about 8% by weight. The toner also comprises as external surface additive package including 4.2% by weight HMDS treated silica (NA50HS, available from Degussa-NAC Corporation) with a 40 nanometer average particle diameter, 0.9% by weight decyltrimethoxysilane (DTMS) treated titania with a 40 nanometer average particle diameter (SMT-5103, available from Tayca Corporation), and 0.5% by weight Zinc Stearate L available from Ferro Corporation.

The toner has a volume median particle size of about 8.3  $\mu\text{m}$ , with percent fines less than 5  $\mu\text{m}$  of no more than 15% by number as measured by a Coulter Counter.

This toner is formed into a developer by combining with a carrier comprised of a 80  $\mu\text{m}$  steel core (supplied by Hoeganaes North America Corporation) coated with 1% by weight PMMA (supplied by Soken) at 200° C.

## Examples 1-4 and Comparative Example 2

## Black Toner with Calcium Stearate

Black toners are prepared as in Comparative Example 1, except that the external surface additive package is changed. In these formulations, the external surface additive package includes 4.3% by weight polydimethylsiloxane (PDMS) treated silica with a 40 nanometer average particle diameter (RY50, available from Nippon Aerosil), 0.9% by weight isobutyltrimethoxysilane (I-BTMS) treated titania with a 40 nanometer average particle diameter (STT100H, available from Titan Kogyo Kabushiki Kaisha (IK Inabata America Corporation, New York)), and varying amounts of Calcium Stearate. The amounts of calcium stearate used are 0 wt % (Comparative Example 2), 0.05 wt % (Example 1), 0.1 wt % (Example 2), 0.25 wt % (Example 3), and 0.5 wt % (Example 4).

The toners have a volume median particle size of about 8.3  $\mu\text{m}$ , with percent fines less than 5  $\mu\text{m}$  of no more than 15% by number as measured by a Coulter Counter.

The toners are formed into developers by combining with a carrier comprised of a 80  $\mu\text{m}$  steel core (supplied by Hoeganaes North America Corporation) coated with 0.2% (by wt.) of methylsilsesquioxane Silicone Resin and 1.0% (by wt.) PMMA (supplied by Soken) at 200° C.

## Triboelectric Charge Sensitivity to Relative Humidity

After the toner compositions are formed, the triboelectric charge on the toner particles is determined by the known Faraday Cage process. The developers are aggressively mixed in a paint shaker (Red Devil 5400, modified to

## 12

operate between 600 and 650 RPM) for a period of 20 minutes. It is believed that this process simulates a mechanical energy input to a toner particle equivalent to that applied in a xerographic housing environment in a low toner throughout mode, that is, a xerographic housing producing a print in which from about 0 to about 2 percent of the print is covered by toner developed from that housing for a period of about 100 to about 10,000 impressions. The triboelectric charge is measured for the developers conditioned in three zones—A-zone (80° F./80% RH), B-zone (70° F./50% RH) and J-zone (70° F./10% RH). The results are shown in FIG. 1.

Comparison of the results of Comparative Example 1 with Comparative Example 2 and Examples 1-4 shows that substitution of the external additive package of the invention for the external additive package of Comparative Example 1 provides significant improved results. In particular, the external additive package of the invention, at increasing amounts of calcium stearate, provides a narrower range of variation (sensitivity) of the triboelectric charge across the A, B and J zones. For example, the toner of Comparative Example 1 exhibits a very strong sensitivity of triboelectric charge to relative humidity, having a sensitivity ratio of 3.3 for J-zone to A-zone and 1.6 for J-zone to B-zone. In contrast, the toners of the invention exhibit a much smaller sensitivity ratio at calcium stearate levels of as low as 0.1 wt %, having a sensitivity ratio of only 1.7 for J-zone to A-zone and only 1.1 for J-zone to B-zone.

## Triboelectric Charge Sensitivity to Toner Age

The triboelectric charge on the toner particles is also determined as a function of simulated toner age. As a surrogate of toner age or residence time in a xerographic housing, the developers are aggressively mixed in a paint shaker (Red Devil 5400, modified to operate between 600 and 650 RPM) for periods of 2, 5, 10, 20, 40 and 60 minutes. The triboelectric charge is measured for the developers conditioned at B-zone, that is, 70 degrees F. and 50% relative humidity. The results are shown in FIG. 2.

Comparison of the results of Comparative Example 1 with Comparative Example 2 and Examples 1-4 shows that substitution of the external additive package of the invention for the external additive package of Comparative Example 1 provides significant improved results. In particular, Comparative Example 1 shows an initial increase in triboelectric charge (up to about 20 minutes), after which it slowly degrades. Comparative Example 2 shows an initial high value of triboelectric charge, but which steadily decreases over time. However, Example 1 (0.05% calcium stearate) shows almost no triboelectric charge response over time, providing an almost ideal function. Examples 2-4, with higher levels of calcium stearate, show a slight rise in triboelectric charge response over time, which rate of rise tends to increase as the calcium stearate loading level increases.

## Example 5

## Cyan Toner with Calcium Stearate

A cyan toner is prepared following the procedures of Comparative Example 1, except that it contains 12.7% by weight of a dispersion of PV Fast Blue in SPARII (3.8% by weight pigment loading total) in a propoxylated bisphenol A fumarate resin having a gel content of about 8% by weight. The toner also comprises as external surface additives 3.3% by weight polydimethylsiloxane (PDMS) treated silica with

## 13

a 40 nanometer average particle diameter (RY50, available from Nippon Aerosil), 0.9% by weight isobutyltrimethoxysilane (I-BTMS) treated titania with a 40 nanometer average particle diameter (STT100H, available from Titan Kogyo Kabushiki Kaisha (IK Inabata America Corporation, New York)), and 0.1% by weight Calcium Stearate.

The toner has a volume median particle size of about 8.3  $\mu\text{m}$ , with percent fines less than 5  $\mu\text{m}$  of no more than 15% by number as measured by a Coulter Counter.

The toner is formed into developers by combining with a carrier comprised of a 80  $\mu\text{m}$  steel core (supplied by Hoechst AG North America Corporation) coated with 0.2% (by wt.) of methylsilsesquioxane Silicone Resin and 1.0% (by wt.) PMMA (supplied by Soken) at 200° C.

## Example 6

## Magenta Toner with Calcium Stearate

A magenta toner is prepared following the procedures of Comparative Example 1, except that it contains 26.3% by weight of a dispersion of Lureton Pink in SPARII (7.9% by weight pigment loading total) in a propoxylated bisphenol A fumarate resin having a gel content of about 8% by weight. The toner also comprises as external surface additives 4.3% by weight polydimethylsiloxane (PDMS) treated silica with a 40 nanometer average particle diameter (RY50, available from Nippon Aerosil), 0.9% by weight isobutyltrimethoxysilane (I-BTMS) treated titania with a 40 nanometer average particle diameter (STT100H, available from Titan Kogyo Kabushiki Kaisha (IK Inabata America Corporation, New York)), and 0.1% by weight Calcium Stearate.

The toner has a volume median particle size of about 8.3  $\mu\text{m}$ , with percent fines less than 5  $\mu\text{m}$  of no more than 15% by number as measured by a Coulter Counter.

The toner is formed into developers by combining with a carrier comprised of a 80  $\mu\text{m}$  steel core (supplied by Hoechst AG North America Corporation) coated with 1.0% (by wt.) PMMA (supplied by Soken) at 200° C.

## Example 7

## Magenta Toner with Calcium Stearate

A magenta toner is prepared following the procedures of Comparative Example 1, except that it contains 26.3% by weight of a dispersion of Lureton Pink in SPARII (7.9% by weight pigment loading total) in a propoxylated bisphenol A fumarate resin having a gel content of about 8% by weight. The toner also comprises as external surface additives 4.3% by weight polydimethylsiloxane (PDMS) treated silica with a 40 nanometer average particle diameter (RY50, available from Nippon Aerosil), 0.9% by weight isobutyltrimethoxysilane (I-BTMS) treated titania with a 40 nanometer average particle diameter (STT100H, available from Titan Kogyo Kabushiki Kaisha (IK Inabata America Corporation, New York)), and 0.2% by weight Calcium Stearate.

The toner has a volume median particle size of about 8.3  $\mu\text{m}$ , with percent fines less than 5  $\mu\text{m}$  of no more than 15% by number as measured by a Coulter Counter.

The toner is formed into developers by combining with a carrier comprised of a 80  $\mu\text{m}$  steel core (supplied by Hoechst AG North America Corporation) coated with 1.0% (by wt.) PMMA (supplied by Soken) at 200° C.

## 14

## Example 8

## Yellow Toner with Calcium Stearate

5 A yellow toner is prepared following the procedures of Comparative Example 1, except that it contains 23.3% by weight of a dispersion of Sunbrite Yellow in SPARII (7.0% by weight pigment loading total) in a propoxylated bisphenol A fumarate resin having a gel content of about 8% by weight. The toner also comprises as external surface additives 3.3% by weight polydimethylsiloxane (PDMS) treated silica with a 40 nanometer average particle diameter (RY50, available from Nippon Aerosil), 0.9% by weight isobutyltrimethoxysilane (I-BTMS) treated titania with a 40 nanometer average particle diameter (STT100H, available from Titan Kogyo Kabushiki Kaisha (IK Inabata America Corporation, New York)), and 0.1% by weight Calcium Stearate.

The toner has a volume median particle size of about 8.3  $\mu\text{m}$ , with percent fines less than 5  $\mu\text{m}$  of no more than 15% by number as measured by a Coulter Counter.

The toner is formed into developers by combining with a carrier comprised of a 80  $\mu\text{m}$  steel core (supplied by Hoechst AG North America Corporation) coated with 0.3% (by wt.) of methylsilsesquioxane Silicone Resin and 1.0% (by wt.) PMMA (supplied by Soken) at 200° C.

While the invention has been described in detail and with reference to specific embodiments thereof, it will be apparent to one skilled in the art that various changes and modifications can be made therein without departing from the spirit and scope thereof.

What is claimed is:

1. A toner composition comprising:

a binder,

a colorant, and

a surface additive package comprising a polydimethylsiloxane surface treated silica, a surface treated titania surface treated with a material selected from a group consisting of decylsilane, decyltrimethoxysilane and isobutyltrimethoxysilane, and calcium stearate, wherein said toner composition comprises from 1 to about 5 weight percent polydimethylsiloxane surface treated silica, from about 0.2 to about 1.5 weight percent surface treated titania, and about 0.05 to about 0.5 weight percent calcium stearate.

2. A toner composition according to claim 1, wherein said toner composition comprises from about 2.3 to about 4.3 weight percent polydimethylsiloxane surface treated silica, from about 0.4 to about 0.9 weight percent surface treated titania, and from about 0.1 to about 0.2 weight percent calcium stearate.

3. A toner composition according to claim 1, wherein said polydimethylsiloxane surface treated silica is a polydimethylsiloxane surface treated fumed silica.

4. A toner composition according to claim 1, wherein said polydimethylsiloxane surface treated silica is selected such that in a low humidity environment, as a concentration of the polydimethylsiloxane surface treated silica decreases, a triboelectric charge of said toner composition decreases, while in a high humidity environment, as the concentration of the polydimethylsiloxane surface treated silica increases, the triboelectric charge of said toner composition increases.

5. A toner composition according to claim 1, wherein said polydimethylsiloxane surface treated silica is present in an amount of from about 1 to about 3.3 percent by weight.

**15**

6. A toner composition according to claim 1, wherein said polydimethylsiloxane surface treated silica is the only xerographically active silica present in the toner composition.

7. A toner composition according to claim 1, wherein said surface treated titania is present in an amount of from about 0.2 to about 0.9 percent by weight.

8. A toner composition according to claim 1, wherein said calcium stearate has a purity of greater than 85%.

9. A toner composition according to claim 1, wherein said calcium stearate is present in an amount of from about 0.05 to about 0.2 percent by weight. 10

10. A toner composition according to claim 1, wherein said calcium stearate is the only metal carboxylate present in the toner composition. 15

11. A toner composition according to claim 1, wherein said calcium stearate is the only metal stearate present in the toner composition.

12. A toner composition according to claim 1, wherein said toner composition has a triboelectric charge from about 10  $\mu$ C/g to about 60  $\mu$ C/g. 20

13. A toner composition according to claim 1, wherein the colorant is selected from the group consisting of black, cyan, magenta, yellow, red, orange, green, and violet.

**16**

14. A developer comprising:  
the toner composition of claim 1, and  
a carrier.

15. A process for preparing a toner composition, comprising:

mixing a resin and a colorant to form toner particles, and applying to an external surface of said toner particles, a surface additive package comprising a polydimethylsiloxane surface treated silica, a surface treated titania surface treated with a material selected from the group consisting of decylsilane, decyltrimethoxysilane and isobutyltrimethoxysilane, and calcium stearate, wherein said toner composition comprises from 1 to about 5 weight percent polydimethylsiloxane surface treated silica, from about 0.2 to about 1.5 weight percent surface treated titania, and about 0.05 to about 0.5 weight percent calcium stearate.

16. A process according to claim 15, wherein said polydimethylsiloxane surface treated silica is the only surface treated silica introduced into the toner composition during the applying of the surface additive package to the external surface of the toner particles.

\* \* \* \* \*